

Aug. 24, 1948.

F. R. HENSEL ET AL

2,447,979

COPPER BASE ALLOY FOR METAL EVAPORATION

Filed July 6, 1944



*Fig. 2*



*Fig. 3*



INVENTORS  
Franz R. Hensel  
BY Earl J. Larsen  
Chester F. Carlson

ATTORNEY

## UNITED STATES PATENT OFFICE

2,447,979

## COPPER BASE ALLOY FOR METAL EVAPORATION

Franz R. Hensel and Earl I. Larsen, Indianapolis,  
Ind., assignors to P. R. Mallory & Co., Inc.,  
Indianapolis, Ind., a corporation of Delaware

Application July 6, 1944, Serial No. 543,634

2 Claims. (Cl. 75—153)

1

This invention relates to improvements in metal evaporation.

An object of the invention is to improve the evaporation of copper and its alloys.

Other objects of the invention will be apparent from the description and claims.

Figure 1 is a sectional elevation of a metal evaporation apparatus;

Figure 2 is a fragmentary cross-section of the tungsten filament coated with the metal to be evaporated; and

Figure 3 shows a wire loop of the metal.

The vaporization process for depositing silver, copper and other metals has been known for some time and used commercially to some extent. The processing as applied to silver is described in considerable detail in the book "Silver in Industry" edited by Lawrence Addicks (Reinhold 1940), pages 291 to 296.

In carrying out the process the metal to be evaporated is usually hung on a tungsten filament as small loops of wire. Electric current is then passed through the filament to heat it and the wire loops are melted and the fused metal clings to the filament and evaporates as the heating is continued. One difficulty which has been encountered with silver and copper has been the failure of these metals to wet the tungsten sufficiently to cling to it during the vaporization process. The metal tends to ball up and drop off the filament before it can be evaporated. It also sometimes tends to spatter during evaporation, probably due to the accumulation of the liquid metal in large globules.

We have now discovered that this difficulty can be overcome in the case of copper and satisfactory wetting of the tungsten filament obtained by adding a small percentage of lithium to copper or its alloys. For example, an alloy of

|          | Per cent | 40 |
|----------|----------|----|
| Lithium  | .05      |    |
| Platinum | 5.00     |    |
| Copper   | Balance  |    |

was found to wet the tungsten extremely well and to give no spattering during evaporation while a similar alloy without the lithium content was found to operate erratically.

In general the amount of lithium which should be alloyed with the copper may fall within the range of .001 to 1%. Other alloying ingredients may be present in the copper. Platinum and palladium in proportions ranging from .25 to 20% are sometimes desirable for improving the wettability still further. In some cases nickel, cobalt

5 or iron may be present in percentages ranging from .001 to .5%.

Referring to the drawing, Figure 1 shows a metal vaporization apparatus comprising a bell jar 10 resting on a pump plate 11 with a rubber gasket 12 between them to afford a gas seal. The bell jar is connected to a vacuum pump through pipe 13 and a Pirani gauge 14 may be provided to measure the degree of vacuum obtained.

10 The articles to be coated with a thin film of copper such as glass plates or mirror blanks 15 are mounted on the inside wall of a cylindrical container 16 supported within the bell jar. The tungsten filament 17 is mounted axially within the 15 container and connected to insulated terminals 18 and 19.

15 The copper alloy to be evaporated is hung on the spiral tungsten filament as little wire loops 20 (Fig. 3) so that when the filament heats up 20 the loops will melt and cling to the filament.

Figure 2 is a fragmentary cross-section of the tungsten filament 17 coated with the fused alloy 21 of copper preparatory to evaporation.

25 While specific embodiments of the invention have been described, it is intended to cover the invention broadly within the spirit and scope of the appended claims.

What is claimed is:

1. An alloy loop for metal evaporation formed of an alloy composed of .001 to 1% lithium, .25 to 20% of a metal selected from the group consisting of platinum and palladium and the balance copper.
2. An alloy wire for metal evaporation composed of about .05% lithium, 5% platinum and the balance copper.

FRANZ R. HENSEL.  
EARL I. LARSEN.

## REFERENCES CITED

The following references are of record in the file of this patent:

## UNITED STATES PATENTS

| 45 | Number    | Name           | Date           |
|----|-----------|----------------|----------------|
|    | 1,291,106 | Payne          | Jan. 14, 1919  |
|    | 1,923,955 | Smith          | Aug. 22, 1933  |
|    | 2,178,233 | Klatzow        | Oct. 31, 1939  |
| 50 | 2,196,302 | Hensel et al.  | Apr. 9, 1940   |
|    | 2,213,312 | Hensel         | Sept. 3, 1940  |
|    | 2,330,062 | Lempert        | Sept. 21, 1943 |
|    | 2,413,604 | Colbert et al. | Dec. 31, 1946  |
|    | 2,413,606 | Colbert et al. | Dec. 31, 1946  |